

Nov. 2, 1937.

F. SCHICK ET AL

2,097,989

PROCESS OF CRACKING HYDROCARBONS BY MEANS OF CATALYSTS

Filed June 8, 1933



INVENTORS

F. SCHICK  
E. EMILUS

*A. B. Wilcox & Co.*

ATTORNEYS

## UNITED STATES PATENT OFFICE

2,097,989

PROCESS OF CRACKING HYDROCARBONS  
BY MEANS OF CATALYSTS

Friedrich Schick and Eugen Emilius, Berlin-Mariendorf, Germany, assignors to the Firm Deutsche Erdöl-Aktiengesellschaft, Berlin-Schöneberg, Germany

Application June 8, 1933, Serial No. 674,945  
In Germany June 9, 1932

4 Claims. (Cl. 196—52)

It is old to conduct hydrocarbons in gaseous form, if required in conjunction with carrying gases or steam, over coke residues of various kinds, such as pit coal coke, semi-coke or lignite coke, or activated charcoal. In particular it has been suggested to transform or "crack" hydrocarbon mixtures with high boiling points, such as mineral oils, tars and similar substances, into products with low boiling points, as for instance 5 motor fuel or gasoline.

The feasibility of such cracking processes is, however, adversely influenced on the one hand by the fact that the catalysts in part possess merely a limited cracking capacity; on the other 15 hand, by the fact that the starting materials or the mode of operating upon them would prove too expensive for obtaining highly active catalysts therefrom, and finally by the fact that the effectiveness of the catalysts rapidly declines in use. 20 The regeneration of the catalysts by gases and vapours merely insures a limited degree of effectiveness, which also drops off within a short time.

We now have found, that the capability of the coke residues for cracking hydrocarbons is very 25 considerably enhanced not only with regard to the initial activity, but also to the duration of efficiency by a far reaching elimination of the ash content of the coke residues obtained from mineral coals. The elimination of the ash content 30 may be effected by treatment with acids, e. g. hydrochloric acid, and by the extraction with water.

Further we have found, that such a treatment 35 will be more effective, if it is carried out in conjunction with an activation by means of suitable gases or vapours, and especially after such a treatment. The reason for the favourable effect of the elimination of ash in conjunction with a previous activation may possibly be looked for, 40 on the one hand, in the fact that the ash-containing coke will be much more activated than the coke from which the ash has been previously eliminated, owing to the intensification of the reaction of the carbon (particularly that with steam) by the ash, and, on the other hand, in that by the previous activation, probably mainly 45 in consequence of a reduction, the ash content becomes more soluble and the coke is rendered more accessible to the extraction means for the elimination of ash due to the increased porosity of the activated coke. The treatment by means of steam at temperatures up to 650° C. was found 50 to be a favourable one for the elimination of ash and simultaneously for the activation.

55 We have further found that it is particularly

advantageous to start, in the characterized production of cracking catalysts, from such distillation residues or coke residues which have been obtained under moderate conditions and also in avoiding local overheating, for which purpose especially the smouldering process or process of incomplete combustion working with scavenging gases under the conditions of low temperature or distillation by internal heating by means of a current of hot inert gas may be employed.

The indicated combined treatment of activation by means of water vapour with subsequent elimination of the ash of the coke renders it also possible, if a sufficiently firm coke is used as starting material, to produce firm, large-sized cracking catalysts up to approximately the size of the original coal briquette used, e. g. 38 x 50 x 50 millimeters, said catalysts possessing a low percentage of ash, for instance only 4%, and a high cracking activity. A cracking catalyst of such kind may, for instance, be obtained by means of a certain addition of caking to non-caking coal, or by the employment of other, also liquid, solidifying agents, such as asphalt, or by drying the starting coal so as to have a lower percentage of water than the ordinary briquettes placed on the market, or else by employing such pit coal or brown coal or lignite, which by their nature furnish particularly firm coke.

The method of carrying through the process 30 and the advantages connected therewith will be elucidated by means of the following examples of execution and comparative experiments:

Semi-coke from brown coal or lignite of Central German origin mined in the district south of Borna, obtained in a large coking or distillation plant at a temperature of about 550° C. by means of scavenging or inert gas, screened down to a grading of 4-7 mms. diameter and having a content of ash of 18%, 1% of which consists of 35 alkalies and 40% of which consists of alkaline earths, is treated at 625° C. with well distributed steam until the capacity of methylene blue absorption of the material has been increased 40 to 15 times the original amount, i. e. during about 2-3 hours. By extracting with aqueous hydrochloric acid and washing with water in conjunction with partial neutralization with ammonia, the ash is reduced down to a residual percentage of ashes of about 5%. Subsequently the obtained coke product is dried at a temperature of about 45 400° C.

With the aid of the catalyzing material thus obtained, the cracking of oils of different kinds 50 can be carried out in such a manner that, after 55

preliminarily heating to about 350° C., they are atomized by means of 50% of superheated steam, their temperature being raised thereby to about 400° C. and by further admixture of gases free from oxygen to about 450° C. The direct heating of the mixture of oil and steam may for instance be effected by means of the flue gases of a burner heated by weak gases, the flame temperature of said flue gases of about 1100° C. being cooled down to about 550° C. with the aid of water or steam sprayed in. The oil vapour, being diluted about twentyfold by steam and flue gases, passes through the chamber containing the catalyst at a velocity of about 4 to 5 liters (at 450° C.) per square centimeter of the cross section and per minute, the temperature of said chamber being maintained at a constant level by indirect heating by means of an electric current or gas circulation. By a single passage of a gas oil having a specific gravity of .845 through a catalyzing path of 70 centimeters length, 40% of gasoline is obtained. When three such catalyzing paths are arranged in series and the gasoline formed is intermediately withdrawn, a total yield of about 60% gasoline and 20% of residual oil is obtained. In the same manner 50% of gasoline and 20% of residual oil may be obtained from a heavy petroleum fraction (specific gravity .900).

In a similar manner, lignite tar-oil of .845 specific gravity preliminarily treated by the so-called Edeleanu process, may be processed continuously with only the addition of steam to the starting oil, using a semi-coke or coke breeze freed from ashes down to 3.2% by means of hydrofluoric acid as splitting catalyst, the yield of gasoline even after several days of working, showing a decrease of only 10% compared with the average yield of 35%. The feed of oil in this process needs only to be interrupted for short periods, during which intervals steam alone is conducted over the catalyst at a temperature of about 600° C.

The ameliorating influence of the elimination of the ashes upon the cracking activity of the catalysts is proved for instance by the comparison of the gasoline production from the above mentioned refined lignite tar-oil when it is performed under identical conditions with the only difference, that in the one case an activated semi-coke free from ashes is employed whereas in the second case a cracking catalyst is used which has been produced in the same manner, from which, however, the ashes have not been eliminated. An average increase of 75% of gasoline output is obtained in the first case, e. g. from 23% to 40% for a catalytic path of 70 centimeters length and a temperature of about 450° C. Even greater increases in yield may yet be observed.

The further, still more valuable progress attained with the aid of the present process, viz, the better maintenance of the activity of the catalyst, is manifested in the above mentioned continuous experiment with refined lignite tar-oil by the fact, that, when employing a catalyst freed from ashes, a waste of only 10% is recorded, whereas when employing a catalyst from which the ashes have not been eliminated, this waste rises to about 35%. The greater durability of the catalysts low in ash content have proved themselves, using the most varied starting materials and under varying conditions, even more conclusively than in the foregoing example.

The influence of the kind of the dry distilla-

tion process, employed for the starting materials, upon the cracking efficiency of the coke residues obtained thereby, is shown for instance by the yields of gasoline which are attained by the employment of cracking catalysts prepared in the same manner from different coke products and used under identical cracking conditions for the treatment of the above mentioned refined lignite tar-oil: When a brown coal or lignite coke is employed as starting material which was obtained in a Rolle plant or kiln at a temperature of about 750° C. or in gas retorts at a temperature of about 850° C., only 50 to 70% of those yields are attained even in the beginning of the cracking operation, which will otherwise be attained when employing cracking catalysts prepared from coke residues obtained under low temperature conditions by means of scavenging gases.

Also in the activation process the employment of higher temperatures appears to be unfavourable for the purposes in question. For instance the use of a low temperature coke, activated with steam at 850° C. and subsequently freed from ashes reduces the yield of cracking products by about 30% when compared with that obtained by means of a cracking catalyst activated at a temperature of only 625° C. but otherwise prepared under identical conditions. The fact that the cokes produced or subsequently treated at a higher temperature are of less suitability for the purposes mentioned herein, will be caused by that the process of elimination of the ashes therefrom is rendered more difficult by said higher heating temperatures. Thus the elimination of the ashes under identical conditions after activation with steam from the previously mentioned brown coal or lignite coke produced at a temperature of 850° C. causes the percentage of ashes to drop from 21 to 7% and for a high temperature coke obtained from bituminous pit coal from 12 to 8%, whereas for a semi-coke or coke breeze gained from brown coal or lignite under low temperature conditions by means of scavenging gases the percentage of ashes drops from 40 to 4%.

The importance of the advantage which will be attained if the activation with steam precedes the elimination of the ashes, is proved by the fact that, starting from the same brown coal or lignite semi-coke or coke breeze the immediate elimination of the ashes will leave a residue of 11% of ashes in the coke, whilst the same method of eliminating the ashes after the activation with steam will reduce this ash content to 4%, although the preliminary activation brings about in the first instance even an enrichment of ashes.

For the purpose of supplementing the data recorded in the foregoing, the following general indications concerning the method of carrying out the present process are given.

Well adapted conditions are: the use of cracking temperatures of from 300° to 500° C.; lengths of the catalyst path between 6 and 0.3 meters; the use of steam up to 200% as accompanying gas; the use of linear velocities from 50 to 300 liters per m<sup>2</sup>/sec. (referred to 20° C.) for the mixture of oil and steam to be treated.

The increase of capacity of the cracking device may be still further enhanced very considerably by limiting the quantity of the accompanying gas, and it has been found that, provided a suitable velocity is used, oil vapour alone may be employed, a satisfactory yield of gasoline nevertheless being obtained. For instance, in conjunction with the

above mentioned gas-oil, an average yield of gaso-line of about 25% was ascertained when using a linear velocity of 6t/m<sup>2</sup>/h and a temperature of 450° C. for a catalytic path of 0.7 meter length.

5 If no steam or the like is to be admixed or only a small quantity thereof, the oils may be finely divided by means of an atomizer, or, after being preliminarily heated with the aid of a tubular heater they may be evaporated in a boiler, simultaneously eliminating the distillation residues.

10 The attached drawing shows one embodiment of the device, partly in section, to be employed for executing the described process, wherein pre-heated oil is brought to cracking temperature either directly by means of steam or by indirect heating.

15 In this drawing 9 is an oil pump, 1 a preheater coil for the hydrocarbon oil to be treated, 7 a pipe for introducing steam, 8 a pre-heater coil for the steam, 2 a superheating device for the steam, and 3 the chambers for cracking the oil to be treated, said chambers being filled with the contact material or catalyst 5 in question. In the embodiment shown three chambers 3 are arranged the one vertically above the other, said chambers being connected with one another by the connecting pipes shown, which contain three-way cocks in such an arrangement that the three chambers may be connected in series or parallel to one another at will, as desired. The catalyst 5 is arranged on perforated members 10 within the chambers 3, and its grains have a size of about 5 to 10 millimeters in diameter. The temperatures are kept constant by means of electrical heating elements 6 and the temperature is measured by thermo-couples 4. The oil or oil and vapour are introduced into the chambers 3 by means of mixing or pressing nozzles, not shown. The device allows one or two of the chambers 3 to be set out of operation for the purpose of regenerating the catalyst contained therein, whereas the others or the other chamber, respectively, remain in operation during this time. A special pipe may be arranged for the removal of the vapour employed for regenerating the catalyst within said chambers.

20 Furthermore, the oils may be de-sulphurized in vaporized state in a known manner prior to entering the catalytic zones, or even between some of these zones or after leaving them. Moreover, substances having the tendency to polymerize, or, if necessary, coarse particles may be removed before entering or between the cracking zones, by passing the vapours over used cracking catalysts or other porous bodies, preferably such, whose cracking activity is of a low degree. It may further prove of advantage, to withdraw from between the separate catalytic steps certain portions of the reaction mixture and, respectively or, add carrier gases or oils or oil vapours to the re-action mixture.

25 The activation prior to the elimination of the ashes may also be effected with the aid of an impregnation by means of alkalis or alkaline earth bases, preferably the former. The elimination of the ashes may be effected in steps by several, different means, e. g. different acids, if desired also with water only. The elimination of the ashes may also be extended to the removal of the silicic acid, e. g. by means of hydrofluoric acid. The washing out of residues of the acid added for the purpose of eliminating the ashes, may be limited or may even be omitted altogether and the acid be treated with volatile salts or bases generating volatile salts and afterwards removed, e. g. by

being heated for instance during the drying of the coke residues freed from ashes.

30 The elimination of the ashes with the aid of sulphuric acid, which embodies certain advantages, may be carried through in such a manner, 5 that after the characterized activation with steam the product is first extracted with water, then treated, with diluted sulphuric acid, subsequently is reduced by means of steam or water-gas or by both, and the series of operations being 10 closed by another extraction with water. In connection herewith that water-gas may be employed, which is produced in conjunction with the activation by means of steam.

35 If desired, the acids may also be employed in 15 a gaseous state.

It should be pointed out that no connection exists between the methylene blue discolouring and the cracking capacity of the catalysts used, 20 particularly with respect to their ash content.

35 The far-reaching influence of the elimination of the ash upon the catalytic effect in connection with the present process is surprising from several points of view. It is a known fact, that an acceleration of the cracking reactions to be 25 considered quite generally takes place on bodies providing a large surface, and several processes utilize this principle by distributing finely divided inorganic oxides and salts, among others, also such, which are precipitated on active coal. The 30 special effect of the preliminarily treated coke or distillation residues by the elimination of the ash was, therefore, not to be expected, because, according to the latest scientific views, on the contrary, a favourable effect of the components 35 of the ash from semi-coke or coke breeze upon the cracking of liquid hydrocarbons, for instance in the manufacture of motor oils and the like from distillation tar, had been assumed. As used in the claims the term "heavy hydrocarbons" 40 has its usual significance in the art, viz., hydrocarbons boiling in the gas-oil range or at higher temperatures.

Having now particularly described and ascertained the nature of our said invention, we declare that what we claim is:—

45 1. The process of cracking heavy hydrocarbons to produce lower boiling hydrocarbons comprising preliminarily purifying said heavy hydrocarbons and thereafter conducting them while 50 heated over catalytic paths of from 0.3 to 6 meters length at temperatures of from 300 to 500° C. and at a velocity of from 50 to 300 liters per square meter of cross-sectional area of reaction chamber, per second, said catalytic paths being composed of 55 coke residues of mineral coals which have been activated by means of steam at a temperature up to about 650° C. and have a low ash content.

60 2. The process of cracking heavy hydrocarbons to produce lower boiling hydrocarbons comprising preliminarily purifying said heavy hydrocarbons in the presence of admixed gases which remain inert under the employed conditions, and thereafter conducting them while heated over 65 catalytic paths of from 0.3 to 6 meters length at temperatures of from 300 to 500° C. and at a velocity of from 50 to 300 liters per square meter of cross-sectional area of reaction chamber, per second, said catalytic paths being composed of 70 coke residues of mineral coals which have been activated by means of steam at a temperature up to about 650° C. and then have been treated to reduce their ash content to a low value.

75 3. The process of cracking heavy hydrocarbons

to produce lower boiling hydrocarbons, comprising preliminarily purifying said heavy hydrocarbons in the presence of admixed superheated steam, and thereafter conducting them while heated over catalytic paths of from 0.3 to 6 meters length at temperatures of from 300 to 500° C. and at a velocity of from 50 to 300 liters per square meter of cross-sectional area of reaction chamber, per second, said catalytic paths being composed of coke residues of mineral coals which have been activated by means of steam at a temperature up to about 650° C. and have been treated with acids and water to reduce the ash content to a low value.

4. In the process of cracking heavy hydrocarbons to produce lower boiling hydrocarbons, the steps of conducting the hydrocarbons through catalytic paths of from 0.3 to 6 meters length at temperatures of from 300° to 500° C. and at a velocity of from 50 to 300 liters per square meter of cross-sectional area of reaction chamber per second, said catalytic paths being composed of coke residues of mineral coals which have been activated by means of steam at a temperature up to about 650° C. and have a low ash content.

FRIEDRICH SCHICK.  
EUGEN EMILIU.S.